

3,275,568

## LOWER VALENT TITANIUM-ALUMINUM HALIDES

Robert Holroyd Stanley, Hartburn, Stockton-on-Tees, and Derek Howden, Nunthorpe, England, assignors to British Titan Products Company Limited, Billingham, England, a corporation of the United Kingdom

No Drawing. Filed Nov. 13, 1962, Ser. No. 237,346  
Claims priority, application Great Britain, Nov. 13, 1961,

40,569/61

10 Claims. (Cl. 252—442)

The present invention relates to a process for the production of mixtures or compounds containing titanium having a valency lower than four, and in particular to mixtures or compounds of this type wherein the titanium is present as a halide. The mixtures or compounds also contain an aluminium halide.

Lower halides of titanium in which the valency of titanium is less than four, for example, titanium trichloride, are commonly present together with an aluminium halide in polymerisation catalysts of the Ziegler or Natta-type, which are widely used in the polymerisation of unsaturated hydrocarbon compounds such as olefins, for example ethylene and propylene.

These compounds, i.e. lower halides of titanium and aluminium halides, are also of value as additives to the vapour phase oxidation of a titanium tetrahalide to produce pigmentary titanium dioxide, since they act as nucleating agents for the titanium dioxide formed and ensure that the pigmentary product is predominantly rutile.

The production of aluminium halides and lower halides of titanium by the reduction of a tetrahalide with aluminium has been previously described, particularly in relation to the production of Ziegler/Natta-type catalysts. Various methods of carrying out this reduction have been disclosed, for example, by:

- (a) Heating together aluminium and titanium tetrachloride at a temperature of about 200° C.
- (b) Heating together aluminium and titanium tetrachloride in a liquid hydrocarbon at a temperature in the range of about 80° C.—180° C. for long periods.
- (c) Ball milling aluminium and titanium tetrachloride together for prolonged periods at a temperature in the range of about 20° C.—100° C.

These methods have the disadvantage that they are time consuming and/or require special equipment.

It is an object of the present invention to provide a process for the production of mixtures or compounds containing a lower halide of titanium and an aluminium halide.

It is also an object of the invention to provide such a mixture or compound which shows excellent activity when used as a component of a Ziegler/Natta-type catalyst.

Accordingly, the present invention is reducing a titanium tetrahalide with aluminium in the presence of free halogen.

The titanium tetrahalide is preferably titanium tetrachloride and the halogen is preferably chlorine, although other halides and halogens may be used if desired, particularly if a liquid solvent or diluent is used to provide a liquid reaction medium. Normally the halogen will be the same as that combined in the titanium tetrahalide. For example, the use of titanium tetraiodide and iodine is also contemplated.

The amount of tetrahalide used is preferably at least sufficient to react with all the aluminium present, i.e. at least a stoichiometric amount of the tetrahalide. Indeed, it is advantageous to use an excess of the tetrahalide in order to ensure that no free aluminium remains in the reaction product, since this might be undesirable; for ex-

ample, the aluminium might contaminate the polymer produced.

The amount of free halogen present may vary widely. As an example of the amounts of free halogen which may be used, it may be noted that suitable amounts may be within the range from 1 to 50 moles of halogen per 100 moles of titanium tetrahalide. Amounts of at least 3 moles of halogen per 100 moles of titanium tetrahalide are particularly contemplated.

10 The reaction may be carried out if desired in the presence of an added liquid diluent for example hydrocarbons such as aromatic hydrocarbons or chlorinated hydrocarbons. Examples of these are benzene, toluene, chlorobenzene, dichlorobenzene, and tetrachloroethylene.

15 Alternatively, where the tetrahalide is liquid, as in the case of titanium tetrachloride, an excess of this may be used to provide a liquid reaction medium.

20 Since the reaction is exothermic it is normally carried out under reflux to prevent loss of any tetrachloride diluent as the reaction proceeds. The reaction will generally commence at room temperature, usually after a short induction period.

25 If the reaction is carried out with only sufficient titanium tetrahalide to complete the reaction (and without additional diluent) a solid purple mass is formed in the reaction vessel. The addition of further titanium tetrahalide or liquid diluent may cause further reaction within this mass.

30 In the preferred method, the reaction is carried out in the presence of an excess of titanium tetrahalide or other liquid diluent. This decreases the violence of the reaction. A slurry is obtained from which a purple or brown solid may be recovered, for example by filtration or distillation followed by drying of the residue.

35 Since the lower halides of titanium are reactive in the presence of oxygen or moisture the reaction and recovery are advantageously carried out in the absence of oxygen or moisture, e.g. under an inert atmosphere such as nitrogen or argon.

40 A convenient method of introducing the halogen into the reaction mixture is to dissolve it in the titanium tetrahalide or in any liquid diluent. This may be done, for example, by adding it to the titanium tetrahalide or diluent before adding this to the aluminium. Alternatively, the halogen may be added after mixing the aluminium and the titanium tetrahalide (and any additional diluent) in the reaction vessel.

45 It is preferred to use only sufficient halogen to initiate the reaction since an excess of halogen may reduce the yield of titanium trihalide. This may be effected by adding the halogen to the titanium tetrahalide or any diluent before the reaction starts, and then adding no further halogen until the reaction is complete.

50 It is, of course, preferred that the aluminium be present in a finely-divided form to ensure the most rapid and complete reaction.

55 If it is desired to use the product of the reaction as a component of a Ziegler/Natta-type catalyst, the dry material may be recovered by known methods and used in a known manner as a catalyst component. For example, it may be milled, suitably by either dry ball milling or ball milling in a liquid vehicle. Where a liquid vehicle is used this is preferably the liquid in which the polymerisation process is to be carried out. After milling the product may be introduced into a polymerisation vessel and the other component of the catalyst may then be also conveniently introduced into the vessel followed by the unsaturated hydrocarbon that is to be polymerised. Such other component of the catalyst is suitably an organo-metallic compound such as an aluminium alkyl or aluminium alkyl halide and in particular an aluminium trialkyl or triaryl, e.g. triethyl aluminium, tri-n-propyl

aluminium, tri-n-butyl aluminium, or triphenyl aluminium. Alkyl or aryl compounds of other metals in groups 1 to 3 of the Periodic Table may be used if desired.

If it is desired to use the product of this invention in the vapour phase oxidation of a titanium tetrahalide, this may be done, for example, by reacting a calculated proportion of aluminium with an excess of titanium tetrahalide in the presence of halogen and using the product as a feed or as an addition to the feed to the vapour phase oxidation reactor. Under such circumstances both the aluminium halide and the lower halide of titanium present in the mixture form nucleating agents for the titanium dioxide formed during the oxidation process.

The following examples describe some methods of carrying out the process of the present invention.

*Example 1*

To a flask filled with dry argon and fitted with a reflux condenser was added 9 g. of aluminium powder, having a mean particle diameter of about 0.5 micron, followed by 190 g. of redistilled titanium tetrachloride. The titanium tetrachloride had been saturated with chlorine at room temperature, so that it contained about 18 mole percent of chlorine (i.e. 18 moles of chlorine per 100 moles of titanium tetrachloride).

No reaction occurred for about 5 minutes, after which some bubbling was noticed. A violent reaction then occurred with the evolution of a considerable amount of heat. Unreacted titanium tetrachloride vapour was condensed in the reflux condenser and returned to the reaction mixture. As the titanium tetrachloride reacted a dark purple solid was precipitated in the flask.

To the flask was then added 100 g. of dry benzene. A vigorous reaction again occurred, but further additions of benzene produced no further reaction.

The dark benzene slurry was filtered under argon, washed five times with 200 cc. of dry benzene, and then dried by heating for four hours at 100° C. under reduced pressure.

The product was a pink/brown solid. It was weighed, and it was found that the yield was 80% (based on the amount of titanium tetrachloride used) of the theoretical yield if the reaction took place according to the equation



The catalytic activity of the product was tested in the following manner. It was ball milled with a suitable quantity of dry n-heptane for 48 hours; a quantity of the resulting product, equivalent to 6.53 millimoles of titanium, was introduced into a flask, followed by 19.59 millimoles of aluminium triethyl. Propylene was then passed into the flask for three hours, after which the polypropylene formed in the flask was recovered and weighed. The weight of the polypropylene was 45 g.; the catalytic activity of the product was therefore 54.7 moles of propylene per mole of titanium per hour.

This result showed that the product had excellent activity as a polymerisation catalyst.

*Example 2*

An experiment was carried out as described in Example 1, except in the following respects:

- (1) 110 ml. of titanium tetrachloride were used (instead of the 190 g. of Example 1),
- (2) 250 ml. of benzene were used (instead of the 100 g. of Example 1),
- (3) chlorine was bubbled into the reaction mixture for twenty minutes before the reaction began,

and in the estimation of the catalytic activity of the resulting product:

- (4) the quantity of the product taken was equivalent to 9.9 millimoles of titanium (instead of the 6.53 millimoles of Example 1),
- (5) the amount of aluminium triethyl was 19.8 millimoles (instead of the 19.59 millimoles of Example 1).

The catalytic activity of the product was found to be 45 moles of propylene per mole of titanium per hour.

*Example 3*

5 An experiment was carried out as described in Example 1, except in the following respects:

- (1) 330 ml. of titanium tetrachloride were used (instead of the 190 g. of Example 1),
- (2) no benzene was used (instead of the 100 g. of Example 1),
- (3) chlorine was bubbled into the reaction mixture for fifteen minutes before the reaction began,

and in the estimation of the catalytic activity of the resulting product:

- 15 (4) the quantity of the product taken was equivalent to 10.1 millimoles of titanium (instead of the 6.53 millimoles of Example 1),
- 20 (5) the amount of aluminium triethyl was 20.2 millimoles (instead of the 19.59 millimoles of Example 1).

The catalytic activity of the product was found to be 22 moles of propylene per mole of titanium per hour.

*Example 4*

25 An experiment was carried out as described in Example 1, except in the following respects:

- (1) 121 ml. of titanium tetrachloride were used (instead of the 190 g. of Example 1),
- 30 (2) 200 ml. of tetrachloroethylene were used (instead of the 100 g. of Example 1),
- (3) chlorine was bubbled into the reaction mixture for twenty minutes before the reaction began,

and in the estimation of the catalytic activity of the resulting product:

- 35 (4) the quantity of the product taken was equivalent to 9.9 millimoles of titanium (instead of the 6.53 millimoles of Example 1),
- 40 (5) the amount aluminium triethyl was 19.8 millimoles (instead of the 19.59 millimoles of Example 1).

The catalytic activity of the product was found to be 16.4 moles of propylene per mole of titanium per hour.

*Example 5*

45 An experiment was carried out as described in Example 1, except in the following respects:

- (1) 45 grams of aluminium were used (instead of the 9 grams of aluminium of Example 1),
- 50 (2) 605 ml. of titanium tetrachloride were used (instead of the 190 g. of Example 1),
- (3) 1000 ml. of benzene were used (instead of the 100 g. of Example 1),
- (4) chlorine was bubbled into the reaction mixture for seventy minutes before the reaction began,

and in the estimation of the catalytic activity of the resulting product:

- 55 (5) the quantity of the resulting product taken was equivalent to 11.9 millimoles of titanium (instead of the 6.53 millimoles of Example 1),
- (6) the amount of aluminium triethyl was 23.8 millimoles (instead of the 19.59 millimoles of Example 1).

The catalytic activity of the product was found to be 37.5 moles of propylene per mole of titanium per hour.

*Example 6*

To a flask filled with dry argon were added 9 g. of aluminium powder, having a mean particle diameter of about 0.5 micron, followed by titanium tetrachloride. The titanium tetrachloride consisted of 22 ml. saturated with chlorine and then mixed with a further 88 ml. not treated with chlorine; since saturated titanium tetrachloride contains about 18 mole percent of chloride, the titanium tetrachloride added to the aluminium contained about 3.5

mole percent of chloride. To the flask was then added 100 ml. of benzene.

The reaction mixture was left overnight.

The next morning it was found that the titanium tetrachloride had been reduced by the aluminium and a dark purple solid similar to that of Example 1 was present in the reaction mixture.

Useful results can also be obtained by using other titanium tetrahalides in the above examples as starting material, such as titanium tetraiodide.

What is claimed is:

1. In the reaction in a liquid reaction medium of a titanium tetrahalide and aluminium metal to produce a lower valent titanium-aluminium halide composition, the improvement comprising introducing at least 1 mole of free halogen per 100 moles of tetrahalide into said reaction medium and initiating said reaction in the reactive presence of free halogen.

2. A process according to claim 1 in which the amount of free halogen is from 3 to 50 moles per 100 moles of titanium tetrahalide.

3. A process according to claim 1 in which the tetrahalide is liquid and an excess of it is used to provide a liquid reaction medium in the reaction chamber.

4. A process according to claim 1 in which a liquid diluent other than the tetrahalide is introduced into the reaction chamber so as to provide a liquid reaction medium therein.

5. A process according to claim 4 in which the liquid diluent is a hydrocarbon.

6. A process according to claim 5 in which said hydrocarbon is selected from the group consisting of benzene, toluene, chlorobenzene, dichlorobenzene and tetrachloroethylene.

7. A process according to claim 1 in which the titanium tetrahalide is titanium tetrachloride and the free halogen is chlorine.

8. A process for the production of material containing aluminium chloride and lower chloride of titanium, comprising introducing into a reaction vessel aluminium metal, an amount of liquid titanium tetrachloride which is in excess of the amount required to react with all the aluminium metal, and from 1 to 50 moles of free chlorine per 100 moles of titanium tetrachloride, these three reactants being intimately intermingled, reacting the aluminium metal with the titanium tetrachloride in the presence of the free chloride to produce aluminium chloride and lower chloride of titanium, and recovering from the reaction vessel material containing aluminium chloride and lower chloride of titanium.

9. A process according to claim 8 in which there is also introduced into the reaction vessel to provide a liquid reaction medium therein a liquid hydrocarbon diluent.

10. A process according to claim 9 in which the liquid hydrocarbon diluent is selected from the group consisting of benzene, toluene, chlorobenzene, dichlorobenzene, and tetrachloroethylene.

#### References Cited by the Examiner

##### UNITED STATES PATENTS

|           |         |                |          |
|-----------|---------|----------------|----------|
| 2,937,928 | 5/1960  | Hughes et al.  | 23—202   |
| 2,954,367 | 9/1960  | Vandenberg     | 260—94.9 |
| 2,964,386 | 12/1960 | Evans et al.   | 23—202   |
| 3,010,787 | 11/1961 | Tornquist      | 23—87    |
| 3,017,401 | 1/1962  | Bo et al.      | 23—87 X  |
| 3,031,440 | 4/1962  | Kaufman et al. |          |
| 3,032,390 | 5/1962  | Caunt          | 23—51    |
| 3,061,410 | 10/1962 | Toland         | 23—87    |
| 3,079,371 | 2/1963  | Bo             | 260—94.9 |

OSCAR R. VERTIZ, Primary Examiner.

JOSEPH L. SCHOFER, MAURICE A. BRINDISI,  
Examiners.

M. B. KURTZMAN, E. STERN, Assistant Examiners.